



US011410795B2

(12) **United States Patent**  
**Horton et al.**

(10) **Patent No.:** **US 11,410,795 B2**  
(45) **Date of Patent:** **Aug. 9, 2022**

(54) **POWER CABLE WITH CONDUCTOR STRAND FILL CONTAINING RECYCLED CROSSLINKED COMPOUNDS**

(71) Applicant: **PRYSMIAN S.p.A.**, Milan (IT)

(72) Inventors: **David Horton**, Lexington, SC (US); **Tyson Baker**, Lexington, SC (US); **Chris Dekonkoly**, Lexington, SC (US)

(73) Assignee: **PRYSMIAN S.p.A.**, Milan (IT)

(\*) Notice: Subject to any disclaimer, the term of this patent is extended or adjusted under 35 U.S.C. 154(b) by 0 days.

(21) Appl. No.: **17/265,075**

(22) PCT Filed: **Aug. 2, 2018**

(86) PCT No.: **PCT/US2018/045012**

§ 371 (c)(1),  
(2) Date: **Feb. 1, 2021**

(87) PCT Pub. No.: **WO2020/027844**

PCT Pub. Date: **Feb. 6, 2020**

(65) **Prior Publication Data**

US 2021/0304921 A1 Sep. 30, 2021

(51) **Int. Cl.**

**H01B 7/288** (2006.01)  
**H01B 13/32** (2006.01)  
**H01B 7/285** (2006.01)

(52) **U.S. Cl.**

CPC ..... **H01B 7/288** (2013.01); **H01B 13/327** (2013.01)

(58) **Field of Classification Search**

CPC ..... H01B 7/282; H01B 7/288; H01B 7/285;  
H01B 13/327

See application file for complete search history.

(56) **References Cited**

**U.S. PATENT DOCUMENTS**

4,703,132 A 10/1987 Marciano-Agostinelli et al.  
4,791,240 A \* 12/1988 Marin ..... H01B 13/327  
174/23 C  
6,638,589 B1 10/2003 Järvenkylä  
7,744,950 B2 6/2010 Belli et al.  
8,722,787 B2 \* 5/2014 Romick ..... B32B 15/085  
524/504

(Continued)

**OTHER PUBLICATIONS**

International Search Report and Written Opinion dated Sep. 27, 2018 in PCT/US2018/045012 filed on Aug. 2, 2018.

(Continued)

*Primary Examiner* — Hoa C Nguyen

*Assistant Examiner* — Amol H Patel

(74) *Attorney, Agent, or Firm* — Oblon, McClelland, Maier & Neustadt, L.L.P.

(57) **ABSTRACT**

A power cable and a process of manufacturing a power cable, where the power cable includes a core containing stranded electrically conductive wires that are impregnated with a water-blocking composition, wherein the water-blocking composition contains, based on a total weight of the water-blocking composition: (i) a thermoplastic polymer; and (ii) a positive amount of up to 30 wt % of a crosslinked polymer, where the crosslinked polymer is in the form of a powder having a particle diameter less than 900  $\mu\text{m}$  and the crosslinked polymer is dispersed in the thermoplastic polymer.

**16 Claims, 2 Drawing Sheets**



(56)

**References Cited**

U.S. PATENT DOCUMENTS

- 2009/0220817 A1 \* 9/2009 Kato ..... H01B 7/288  
428/626  
2016/0326759 A1 \* 11/2016 Huh ..... E04G 23/0211  
2018/0010850 A1 1/2018 Moore

OTHER PUBLICATIONS

Extended European Search Report dated Feb. 17, 2022 in corresponding European Patent Application No. 18928336.9, 7 pages.  
Office Action dated Apr. 6, 2022, in corresponding Chinese Application No. 201680096200.8 (with English translation).

\* cited by examiner



FIG. 1



FIG. 2



FIG. 3

## 1

**POWER CABLE WITH CONDUCTOR  
STRAND FILL CONTAINING RECYCLED  
CROSSLINKED COMPOUNDS**

**CROSS-REFERENCE TO RELATED  
APPLICATIONS**

Not applicable.

**STATEMENT REGARDING FEDERALLY  
SPONSORED RESEARCH OR DEVELOPMENT**

Not applicable.

**THE NAMES OF THE PARTIES TO A JOINT  
RESEARCH AGREEMENT**

Not applicable.

**INCORPORATION-BY-REFERENCE OF  
MATERIAL SUBMITTED ON A COMPACT  
DISC**

Not applicable.

**STATEMENT REGARDING PRIOR  
DISCLOSURES BY THE INVENTOR OR A  
JOINT INVENTOR**

Not applicable.

**BACKGROUND OF THE INVENTION**

**Field of the Invention**

This disclosure relates to a power cable comprising an electrically conductive core made of a plurality of wires that are stranded and impregnated with a water-blocking composition, where the water-blocking material comprises (i) a thermoplastic polymer and (ii) up to 30 wt % of a recycled crosslinked polymer, based on a total weight of the water-blocking material, and a process for manufacturing said cable cores. This disclosure further relates to power cables comprising said electrically conductive core for use in underground and submarine environments.

**Description of the Related Art**

The penetration of water into the electrically conductive core of a power cable is problematic because the water can vaporize due to the temperatures reached during the use of the conductor and migrate into the insulation of the power cable where "trees" may form potentially causing a decrease in the electrical properties of the insulation and an increased risk of electrical perforation. The water penetration issue is particularly felt in underground and underwater cable deployments where the risks of the entry and spreading of water along the entire cable are very high. Water that penetrates the electrically conductive core is also problematic because it can cause corrosion of the metal wires forming the conductive core.

To prevent the migration along the conducting core of insulated electric cables, U.S. Pat. No. 4,791,240 proposes an electric cable comprising a conductor in the form of a rope constituted by a plurality of metallic wires laid up together and impregnated with a filler that, when extruded, forms a solid and hard compound between the metallic

## 2

wires. The filler compound is based on a polymeric compound having a Mooney viscosity from about 10-60 at 100° C. and a Shore A hardness from about 10-90.

Known water-blocking materials (also referred to as strand fill materials) tend to be expensive and include commodities that fluctuate in price, such as graphite and rubber compounds.

Electric cables comprise layers made of compositions based on crosslinked polymers that are obtained from a peroxide or silane crosslinking process, such as ethylene propylene rubber (EPR), cross-linked polyethylene (XLPE) and optional additives. The waste streams of these cross-linked, partially crosslinked and uncrosslinked scraps thereof are not insignificant. Contrarily to thermoplastic materials, like the strand fill materials, crosslinked and partially crosslinked cannot be re-melted and re-used. Thus, aside from the environmental footprint of these waste streams, production costs are increased because of the disposal of these waste streams.

It would be advantageous to reduce the cost and reliance on known water-blocking materials through the use of cheaper polymeric materials. However, the incorporation of non-thermoplastic materials, such as thermosets and cross-linked polymeric materials, into thermoplastic compositions is problematic because they have different viscosities and this difference in viscosity can result in a heterogeneous mixture potentially affecting the processing conditions needed to ensure complete impregnation of the interstices and, accordingly the cable protection. In the case of the addition of a crosslinked or partially crosslinked recycled polymeric material, reheating cannot achieve softening or melting, thus it would be expected to increase the likelihood of water being able to migrate along the conductive core of the cable due to voids that may form at the interfaces of the thermoplastic water-blocking material and the crosslinked polymeric material. That is, the different phases of the crosslinked polymer and the water-blocking material during the impregnating process would be expected to contribute to interface voids.

U.S. Pat. No. 4,123,584 discloses a process for recovering solid scrap thermosetting types of plastic compounds by: hot granulating the fresh scraps before they fully cure; cooling the granules to avoid further curing; and then, forming a fine powder of about 18 mesh (1 mm) or less from the granules.

U.S. Pat. No. 4,123,584 proposes to use the reclaimed thermosetting compound in insulation coatings for electrical conductors by: extruding the reclaimed compound onto an electrical conductor; curing the coated conductor by passing it through a continuous vulcanization tube; and then cooling the cured, coated conductor. It is essential in U.S. Pat. No. 4,123,584 that the reclaimed thermosetting compound is not entirely cured, although it is indicated that substantially cured compounds may be reused in some less exacting processes, such as injection molding and the extrusion of thick insulation coatings, if it is blended with at least 25 wt % of virgin material.

The exemplary process in U.S. Pat. No. 4,123,584 relates to a blend made of 90 wt % of a very low cured crosslinkable polyethylene and 10 wt % of a reclaimed crosslinked polyethylene. The use of a recycled blend in a water-blocking material is not envisaged nor is recycling of the partially crosslinked thermosetting polymer with a thermoplastic polymer.

U.S. Pat. No. 6,638,589 discloses a method of using recycled plastic material by mixing crosslinked polyethylene with the base material, e.g., a polyolefin, of the product to be produced, in such a way that the proportion of the

recycled crosslinked polyethylene in the mixture is less than 30 wt %. The crosslinked polyethylene is ground by grating and tearing to form a powder that has a grain size of less than 1 mm and that, when extruded, does not melt with the base material and orientates so that its strength continues to grow to some extent. U.S. Pat. No. 6,638,589 exemplifies the formation of plastic pipes from the blend containing the recycled crosslinked polyethylene. U.S. Pat. No. 6,638,589 does not envisage the use of the recycled blend as a water-blocking material or in the manufacture of cables.

#### SUMMARY OF THE INVENTION

An object of the present disclosure is to reduce the cost of manufacturing a power cable having an electrically conductive core comprising a water-blocking composition suitable to prevent ingress and migration of water through the conductive core without substantially altering the cable manufacturing efficiency, for example in term of ease and speed.

Applicant envisaged incorporating an at least partially crosslinked scrap material into the thermoplastic water-blocking material. The reuse of the scrap material reduces the costs of production by decreasing the disposal costs associated with crosslinked polymers obtained from peroxide or silane curing processes and the relative amount of the thermoplastic water-blocking material commonly used in stranding process of the electrically conductive core.

Applicant found that a given amount of an at least partially crosslinked material in admixture with a thermoplastic water-blocking material could be used for fully impregnating the electrical conductor wires of a power cable at an industrially satisfactory manufacturing speed, when the at least partially crosslinked material is in form a powder with a particle diameter of less than 900  $\mu\text{m}$ .

An object of the present disclosure is achieved with a power cable comprising stranded electrically conductive wires that are impregnated with a water-blocking composition comprising:

- (i) a thermoplastic polymer; and
- (ii) a positive amount of up to 30 wt %, based on a total weight of the water-blocking composition, of a cross-linked polymer,

wherein the crosslinked polymer is in the form of a powder having a particle diameter less than 900  $\mu\text{m}$ , and

wherein the crosslinked polymer is dispersed in the thermoplastic polymer.

The present disclosure further relates to a process for manufacturing a power cable, which comprises:

dispersing up to 30 wt % of a crosslinked polymer in the form of a powder having a particle diameter less than 900  $\mu\text{m}$  in a thermoplastic polymer to obtain a water-blocking composition;

pumping the water-blocking composition to impregnate stranded electrically conductive wires, to obtain a cable core;

wherein the pumping is carried out at a line speed greater than 250 RPM (rotation per minute).

#### BRIEF DESCRIPTION OF THE DRAWINGS

A more complete appreciation of the disclosure and many of the attendant advantages thereof will be readily obtained as the same becomes better understood by reference to the following detailed description when considered in connection with the accompanying drawings, wherein:

FIG. 1 is a perspective view of a cable according to the present disclosure.

FIG. 2 is a fragmentary, enlarged cross-section of a cable according to the present disclosure.

5 FIG. 3 is a schematic, side view of a device for carrying out the method for making a cable according to the present disclosure.

#### DETAILED DESCRIPTION OF THE PREFERRED EMBODIMENTS

10 It is to be understood that all the possible combinations of particular features of the objects of the present disclosure are included in this specification. For example, where a particular feature is disclosed in the context of a particular aspect or embodiment, or a particular claim, that feature can also be used, to the extent possible, in combination with and/or in the context of other particular aspects and embodiments, and in the disclosure generally.

20 The numerical ranges in this disclosure are approximate, and thus may include values outside of the range unless otherwise indicated. Numerical ranges include all values from and including the lower and the upper values, in increments of one unit, provided that there is a separation of at least two units between any lower value and any higher value. As an example, if a compositional, physical or other property, such as, for example, molecular weight, viscosity, melt index, etc., is from 100 to 1,000, it is intended that all individual values, such as 100, 101, 102, etc., and sub ranges, such as 100 to 144, 155 to 170, 197 to 200, etc., are expressly enumerated. For ranges containing values which are less than one or containing fractional numbers greater than one (e.g., 1.1, 1.5, etc.), one unit is considered to be 0.0001, 0.001, 0.01 or 0.1, as appropriate. For ranges containing single digit numbers less than ten (e.g., 1 to 5), one unit is typically considered to be 0.1. These are only examples of what is specifically intended, and all possible combinations of numerical values between the lowest value and the highest value enumerated, are to be considered to be expressly stated in this disclosure. Numerical ranges are provided within this disclosure for, among other things, the component amounts of the composition and various process parameters.

45 “Composition” means a mixture or blend of two or more components.

“Polymer” means a compound containing more than 4 monomer units of the same or different type. The term “polymer” includes homopolymers, copolymers, terpolymers, interpolymers, and so on.

50 “Thermoplastic polymer” means a polymer capable of being repeatedly softened by heating and hardened by cooling through a characteristic temperature range, wherein the change upon heating is substantially physical; as opposed to a “thermosetting polymer,” which is a polymer that “sets” irreversibly when cured, typically due to a crosslinking reaction of the constituents, to form a substantially infusible or insoluble product also known as a “thermoset.” Examples of thermoplastic polymers include, by way of illustration only, end-capped polyacetals, such as poly(oxymethylene) or polyformaldehyde, poly(trichloroacetaldehyde), poly(n-valeraldehyde), poly(acetaldehyde), poly(propionaldehyde), and the like; acrylic polymers, such as polyacrylamide, poly(acrylic acid), poly(methacrylic acid), poly(ethyl acrylate), poly(methyl methacrylate), and the like; fluorocarbon polymers, such as poly(tetrafluoroethylene), perfluorinated ethylene-propylene copolymers, ethylene-tetrafluoroethylene copolymers, poly(chlorotrifluoroethylene), and the like.

luoroethylene), ethylene-chlorotrifluoroethylene copolymers, poly(vinylidene fluoride), poly(vinyl fluoride), and the like; polyamides, such as poly(6-aminocaproic acid) or poly(epsilon-caprolactam), poly(hexamethylene adipamide), poly(hexamethylene sebacamide), poly(11-amino-undecanoic acid), and the like; polyaramides, such as poly(imino-1,3-phenyleneiminoisophthaloyl) or poly(m-phenylene isophthalamide), and the like; parylenes, such as poly-p-xylylene, poly(chloro-p-xylylene), and the like; polyaryl ethers, such as poly(oxy-2,6-dimethyl-1,4-phenylene) or poly(p-phenylene oxide), and the like; polyaryl sulfones, such as poly(oxy-1,4-phenylenesulfonyl-1,4-phenyleneoxy-1,4-phenylene-isopropylidene-1,4-phenylene), poly(sulfonyl-1,4-phenyleneoxy 1,4-phenylenesulfonyl-4,4'-biphenylene), and the like; polycarbonates, such as poly(bisphenolA) or poly(carbonyldioxy-1,4-phenyleneisopropylidene-1,4-phenylene), and the like; polyesters, such as poly(ethylene terephthalate), poly(tetramethylene terephthalate), poly(cyclohexylene-1,4-dimethylene terephthalate) or poly(oxymethylene-1,4-cyclohexylenemethyleneoxyterephthaloyl), and the like; polyaryl sulfides, such as poly(p-phenylene sulfide) or poly(thio-1,4-phenylene), and the like; polyimides, such as poly(pyromellitimido-1,4-phenylene), and the like; polyolefins, such as polyethylene, polypropylene, poly(l-butene), poly(2-butene), poly(l-pentene), poly(2-pentene), poly(3-methyl-1-pentene), poly(4-methyl-1-pentene), 1,2-poly-1,3-butadiene, 1,4-poly-1,3-butadiene, polyisoprene, polychloroprene, polyacrylonitrile, poly(vinyl acetate), polystyrene, and the like.

“Crosslinkable” and “curable” mean that the polymer is not cured or crosslinked and has not been subjected or exposed to treatment that has induced substantial crosslinking although the polymer comprises additive(s) or functionality which will cause or promote substantial crosslinking upon subjection or exposure to such treatment.

“Fully cured” or “fully crosslinked” means the polymer/crosslinker system has effectively developed the maximum practical viscosity under the particular conditions of use, unless indicated otherwise or clear from the context within which the term is used. The degree of cure can be described in terms of gel content, or conversely, extractable components. Gel content reported as percent gel is determined by a procedure which comprises determining the amount of insoluble polymer by soaking the crosslinked polymer for 48 hours in organic solvent at room temperature, weighing the dried residue, and making suitable corrections based upon knowledge of the composition. Thus, corrected initial and final weights are obtained by subtracting from the initial weight the weight of soluble components, other than polymer to be crosslinked, such as extender oils, plasticizers and components of the composition that are soluble in the organic solvent. Any insoluble pigments, fillers, and the like are subtracted from both the initial and final weights. Generally, fully crosslinked means that less than 10% by weight of the crosslinked polymer is extractable by an organic solvent. In another embodiment, the amount of organic solvent extractable is less than 5% by weight, less than 3% by weight, less than 2% by weight, or less than 1% by weight. Alternatively, fully crosslinked means that the cross-linked polymer has a gel content of greater than 90%, greater than 95%, greater than 97%, greater than 98%, or greater than 99%.

“Polyolefin” means a polymer containing units derived from at least one type of olefin, typically a C<sub>2</sub>-C<sub>20</sub> olefin, such as ethylene, propylene, butylene, pentene, hexene, octene, etc.

The objects of the present disclosure are obtained by a power cable that comprises a core comprising stranded electrically conductive wires that are impregnated with a water-blocking composition, wherein the water-blocking composition comprises, based on a total weight of the water-blocking composition:

- (i) a thermoplastic polymer; and
  - (ii) a positive amount of up to 30 wt % of at least one crosslinked polymer,
- wherein the crosslinked polymer is in the form of a powder having a particle diameter less than 900 μm, and

wherein the crosslinked polymer is dispersed in the thermoplastic polymer.

#### Thermoplastic Polymer

Examples of the thermoplastic polymers included in the water-blocking composition are based on thermoplastic polyolefins, such as polyethylene homopolymers, polyethylene copolymers (e.g., ethylene-propylene copolymer), isobutylene homopolymers, and isobutylene copolymers, butadiene-styrene copolymers, or on polyesters such as ethyl vinyl acetate polymers.

The amount of the thermoplastic polymer in the water-blocking composition may range from 20 to 90 wt %, from 20 to 85 wt %, from 65 to 85 wt %.

#### Crosslinked Polymer

Crosslinked polymers are relatively immobile when subjected to shear, whereas low viscosity fluids, such as thermoplastic polymers, flow relatively easily. In addition, as the particle diameter of the crosslinked polymer increases and the number of particles decreases, there is less resistance to flow because there are less particle-particle interactions restricting the flow, while decreases in the particle diameter and increases number of particles results in more particle-particle interactions that increase the resistance to flow. Increases in the resistance to flow results in inhomogeneous distributions of the crosslinked polymer in the thermoplastic polymer, which impairs the ability of the water-blocking composition to prevent ingress and migration of water through the conductive core at an industrially acceptable manufacturing speed.

The crosslinked polymer is in the form of a powder having a particle diameter of less than 900 μm. The cross-linked polymer powder is dispersed in the thermoplastic polymer of the disclosure. In certain embodiments, the particle diameter of the powder is from 100 μm to 600 μm, or from 200 μm to 400 μm. The upper limit of the particle diameter of the crosslinked polymer is 900 μm since diameters greater than 900 μm result in defects in the water-blocking composition and impairs its ability to prevent ingress and migration of water through the conductive core.

The crosslinked polymer is included in the water-blocking composition in a positive amount of up to 30 wt %, based on the total weight of the water-blocking composition. In certain embodiments, the content of crosslinked polymer is at least 10 wt % or at least 15 wt %. Although amounts greater than 30 wt % of the crosslinked polyolefin may be included in the water-blocking composition, amounts greater than 30 wt % are unsuitable for an industrially efficient manufacturing process because breakages occur in the water-blocking composition when utilized with line speeds exceeding 250 rotations per minute. In certain embodiments, the upper limit of the crosslinked polymer is 28 wt %, 25 wt %, 22.5 wt %, or 20 wt %. For example, the content of crosslinked polymer included in the water-blocking composition, ranges from 10 wt % to 25 wt % based on a total weight of the water-blocking composition.

The crosslinked polymer may be a recycled crosslinked polymer.

In certain embodiments, the crosslinked polyolefin is a crosslinked polyolefin, for example a homopolymer of ethylene or copolymer of ethylene with one or more comonomers, such as a crosslinked LDPE, VLDPE, LLDPE, MDPE, or HDPE, or a mixture of such polymers. Additional crosslinked polymers include ethylene-propylene rubber (EPR) and ethylene propylene diene rubber (EPDM), ethylene vinyl acetate (EVA), ethylene butyl acetate (EBA), and ethylene ethyl acetate (EEA).

The crosslinked polymer may be crosslinked with a crosslinking agent such as sulfur, peroxide, or a silane. In certain embodiments, the crosslinked polymer is crosslinked via silane groups, where said silane groups can be introduced into the polyolefin structure by copolymerization of monomers, such as olefin monomers, with silane-moiety bearing comonomers, or by grafting crosslinkable silane-moieties bearing compounds, such as unsaturated silane compounds with hydrolysable silane group(s), onto the polyolefin. Grafting is usually performed by radical reaction using free radical generating agents. In both the copolymerization and grafting methods, the unsaturated silane compound may be represented by the formula (I):



wherein:

R is an ethylenically unsaturated hydrocarbyl or hydrocarboxy group;

R' is an aliphatic, saturated hydrocarbyl group;

Y is a hydrolysable organic group, where plural Y groups may be the same or different; and

n is 0, 1, or 2.

Specific examples of the unsaturated silane compound are those in which R is vinyl, allyl, isopropenyl, butenyl, cyclohexenyl, or gamma-(meth)acryloxypropyl, Y is methoxy, ethoxy, formyloxy, acetoxy, propionyloxy, or an alkyl or arylamino group, and R' is a methyl, ethyl, propyl, decyl or phenyl group. For instance, the unsaturated silane compound may have formula  $CH_2=CHSi(OA)_3$ , wherein A is a hydrocarbyl group having 1-8 carbon atoms or 1-4 carbon atoms. Specific silanes include vinyltrimethoxy silane, vinyl dimethoxyethoxy silane, vinyltriethoxy silane, gamma-(meth)acryl-oxypropyl silane, and vinyltriacetoxy silane.

In certain embodiments, the crosslinked polymer is cross-linked via radical reaction with a peroxide. Examples of peroxides used for crosslinking are di-tert-amylperoxide, 2,5-di(tert-butylperoxy)-2,5-dimethyl-3-hexyne, 2,5-di(tert-butylperoxy)-2,5-dimethylhexane, tert-butylcumylperoxide, di(tert-butyl)peroxide, dicumylperoxide, di(tert-butylperoxy-isopropyl)benzene, butyl-4,4-bis(tert-butylperoxy)valerate, 1,1-bis(tert-butylperoxy)-3,3,5-trimethylcyclohexane, tert-butylperoxybenzoate, dibenzoyl-peroxide.

The crosslinking agents (e.g., the unsaturated silane compounds and peroxide compounds), are generally added to the crosslinkable polyolefin in an amount from 0.1 to 10 wt %, or from 0.1 to 5 wt %.

In an embodiment, the thermoplastic polymer and/or the crosslinked polymer of the water-blocking composition can be semiconductive, thus making the water-blocking composition of the disclosure semiconductive. In the case of the crosslinked polymer, it can be a waste material from cable semiconductive layer manufacturing. A semiconductive thermoplastic polymer and/or the crosslinked polymer can contain an electrically conductive filler, such as carbon black or graphite or a mixture thereof.

Representative electrically conductive fillers have a surface area BET greater than 20 m<sup>2</sup>/g, for example of from 40 and 500 m<sup>2</sup>/g.

The electrically conductive filler can be present in the thermoplastic polymer and/or in the crosslinked polymer in an amount suitable to achieve the desired conductivity, which is usually below 1000 ohm·m, below 500 ohm·m, or of about 1 ohm·m. The amount of conductive filler can range from 5 to 50 wt %, for example from 10 to 40 wt %, based on the total weight of the semiconductive thermoplastic polymer or of the semiconductive crosslinked polymer. This amount can depend on the specific conductive feature of the filler, as known to those of skill in the art.

#### Additives

The water-blocking composition may include additives, such as water-swellable material, antioxidants, crosslinking boosters, scorch retardants, processing aids, fillers, crosslinking agents, ultraviolet absorbers, stabilizers, antistatic agents, nucleating agents, slip agents, plasticizers, lubricants, viscosity control agents, tackifiers, anti-blocking agents, surfactants, extender oils, acid scavengers and/or metal deactivators. The content of said additives may ranges from 0 to 10 wt % or from 0 to 5 wt %, based on a total weight of the water-blocking composition.

As for the swellable material, it can be in form of powders based on organic material such as polyacrylates and polyacrylamides, either in se or grafted on natural polymers such as the amides, cellulose and esters of methyl-cellulose and the ethers of cellulose, such as, carboxymethyl cellulose.

#### Water-Blocking Composition

The water-blocking composition may be prepared by mixing the electrically conductive filler and any additives with the thermoplastic polymer, to obtain an electrically conductive thermoplastic composition, and then mixing the crosslinked polymer with the electrically conductive thermoplastic composition using a mixtruder that includes a double arm or a sigma blade mixer with an extruder. Alternatively, the water-blocking composition may be prepared by mixing the electrically conductive filler, any additives, and the crosslinked polymer with the thermoplastic polymer using a mixtruder. The mixture of the crosslinked polymer and the thermoplastic polymer are heated before impregnation of the core comprising stranded electrically conductive wires.

The crosslinked polymer may be a recycled crosslinked polymer. The recycled crosslinked polymer may be obtained from subsequent layers of the power cable described below. The recycled crosslinked polymer can be prepared by shredding and pulverizing a crosslinked polymer and passing the pulverized crosslinked polymer through screen to the desired particle diameter.

Referring now to the drawings, wherein like reference numerals designate identical or corresponding parts throughout the several views.

#### Power Cable

A cable of the present disclosure is illustrated in FIGS. 1 and 2, and comprises (from the inside towards the outside), an electric conductor 1 in the form of a rope comprising a plurality of metallic wires 2 made, for example, of copper, aluminum, or aluminum alloy and which are stranded together.

The individual metallic wires 2, except for those forming the outermost layer of the rope (as shown in FIG. 2), are completely surrounded by a water-blocking composition 3a, which must avoid the moisture penetration and migration along of the electric conductor 1. It is essential that all of the

spaces **3** in-between the metallic wires **2** are completely filled up with the water-blocking composition **3a**.

Typically, an inner semiconductive layer **4** is provided around the electric conductor **1**. The inner semiconductive layer **4** engages the outermost surfaces of the electric conductor **1** and may directly contact the outermost surface of wires **2**. Water swellable material may be applied at the interface between the inner semiconductive layer **4** and the outermost surface of wires **2**. Such water swellable material may be in form of powder, strands or tapes, and may be based on polyacrylates and polyacrylamides, either in se or grafted on polymers such as the amides, cellulose and esters of methyl-cellulose and the ethers of cellulose, such as, carboxymethyl cellulose.

An electrically insulating layer **5** is disposed around the inner semiconductive layer **4**. The electrical insulating layer **5** provides electrical insulation around the cable core **1** and may directly contact the inner semiconductive layer **4**.

An outer semiconductive layer **6** is disposed around the insulating layer **5** and may directly contact the insulating layer **5**.

The inner semiconductive layer **4**, the electrically insulating layer **5**, and the outer semiconductive layer **6** may be coextruded or extruded separate from one another. If extruded separately, the electrically insulating layer **5** is extruded onto the inner semiconductive layer **4** before it cools and then the outer semiconductive layer **6** is extruded onto the electrically insulating layer **5** before it cools to increase the adhesion between the respective layers.

The inner semiconductive layer **4**, the electrically insulating layer **5**, and the outer semiconductive layer **6** comprise at least one polymer selected from the group consisting of a polyethylene homopolymer, a polyethylene copolymer, a polypropylene homopolymer, a polypropylene copolymer. Exemplary polyethylene polymers include low density polyethylene (LDPE), linear low density polyethylene (LLDPE), crosslinked polyethylene (XLPE), ethylene/vinyl acetate (EVA), ethylene butyl acetate (EBA), ethylene ethyl acetate (EEA), ethylene-propylene rubber (EPR), ethylene propylene diene rubber (EPDM). In certain embodiments, the inner semiconductive layer **4**, the electrically insulating layer **5**, and the outer semiconductive layer **6** are all formed of the same polymer, with the proviso that the semiconductive layers comprise a conductive filler and the insulating layer does not. In certain embodiments, at least one of the inner semiconductive layer **4**, the electrically insulating layer **5**, and the outer semiconductive layer **6** comprises a cross-linked polymer that is compositionally the same as the crosslinked polymer in the water-blocking composition.

The inner semiconductive layer **4**, the electrically insulating layer **5**, and the outer semiconductive layer **6** may comprise any of the additives mentioned with respect to the water-blocking composition.

The inner semiconductive layer **4** and the outer semiconductive layer **6** further include a suitable amount of an electrically conductive filler to impart semiconductive properties. The details of the electrically conductive filler are the same as mentioned above with respect to the water-blocking composition.

The insulating layer **5** does not include an electrically conductive filler or in the event that the insulating layer **5** includes an electrically conductive filler, it is included in an amount that does not provide the insulating layer **5** with semiconductive properties. Tree retardant additives can be added to XLPE to inhibit the growth of water trees in the insulation layer.

Together, the inner semiconductive layer **4**, the insulating layer **5**, and the outer semiconductive layer **6** form an insulating system that surrounds the electric conductor **1**. The combination of the electric conductor **1** and the insulating system can be referred to as an insulated conductor.

Around the outer semiconductive layer **6** of the insulated conductor, other per se known elements (not shown) can also be provided, such as, for example, a screen, a water blocking barrier, protective layer(s), armoring layer(s), etc. For instance, a metallic shield comprising a metallic screen or sheath layer may be provided. The metallic screen or sheath layer is made of aluminum, steel, lead, or copper and is in the form of wires, braids, a helically wound tape, or a longitudinally folded foil.

FIG. 3 schematically shows a side elevation view, partly in cross-section, of a device for forming the electric conductor **1**. The device comprises an annular die **7** secured to and coaxial with a cylindrical body which is formed by two parts **8** and **9** which are joined together and which has a through-cavity. The part **8** of the cylindrical body has a cylindrical shaped cavity **10** through which the rope portion **15**, formed in the device, passes. The wires **2**, intended for forming the outermost layer of the rope portion **15** which was produced in the device, and the core **16** of the rope produced previously with an identical device and already impregnated with the water-blocking composition pass through the cavity **11**.

The part **9** of the cylindrical body has a truncated cone shaped inner cavity **11** which, in correspondence to the lesser base thereof, extends to the cavity of the annular die **7**. In the part **9** of the cylindrical body, there is a through-hole **12** communicating with an extruder (not shown) which delivers the water-blocking composition of the present disclosure into the truncated-cone cavity **11**.

The wires **2**, and the core **16** of the rope previously formed and already impregnated with the water-blocking composition, advance in a continuous manner toward the annular die **7**. During said advance, the wires **2** and the core **16** drag along with them the water-blocking composition which the extruder has delivered by means of the through-hole **12** into the truncated-cone cavity **11**, and said composition passes through the wires **2** as they approach the core **16** of the rope.

The water-blocking composition is prevented by the wires **2** and the core **16** from passing through the annular die **7** (where the joining and the compacting of the plurality of wires **2** on the already impregnated core **16** takes place), fills up all the spaces existing between the wires and assuring that at least one layer of the water-blocking composition exists between the wires **2** and the wires which are disposed in the radially outermost portion of said core **16**.

The device of FIG. 3 may also be provided with another through hole **13** (indicated with a broken line) in the part **8** of the cylindrical body which also communicates with the extruder for forming a layer **14** of the water-blocking composition around the already formed portion **15**.

If another layer of wires **2** is to be applied over the structure leaving the device shown in FIG. 3, the other layers of wires **2** may be applied over such structure by a second device the same as the device shown in FIG. 3 and disposed downstream thereof, but if a layer **14** of the water-blocking composition is not to be applied to the exterior of the rope at the second device, the through hole **13** may be omitted.

A cable according to the present disclosure can be manufactured at industrially efficient line speed. In particular the stranded electrically conductive wires of the cable core can

## 11

be impregnated by the present water-blocking composition cable at a line speed greater than 250 RPM, for example of at least 400 RPM.

## Examples

Hot and cold bend water penetration resistance tests were performed in accordance with ANSI/ICEA T-31-610-2014, section 3.2.2.

Example 1. A blend containing a semiconducting thermoplastic water-blocking material (Chase BiH<sub>2</sub>Ock® sold by Chase Wire & Cable Materials, Westwood, Mass.) and 23.0 wt % of pulverized silane crosslinked polyethylene XLPE was prepared with an industrial mixtruder specially designed for the mixing of highly viscous materials. The crosslinked polyethylene XLPE had a particle size of about 295 µm. The mixtruder includes a double arm, or sigma, blade mixer with an extruder to facilitate the removal of the mastic after the mixing has taken place.

The blend was applied to a 42.4 mm<sup>2</sup> (1/0 AWG) conductor by pumping the blend through a heated hose and die at a line speed of 450 RPMs (rotation per minute). An XLPE insulation system was extruded over the so-filled conductor. The cable was left unsheathed for performing the water penetration test.

0.9 m (36") long samples of the above cable were bent around a 20.32 cm (8") diameter drum after performing a 130° C. hot treatment, while other similar samples were bent around a 20.32 cm (8") diameter drum after performing a -10° C. cold treatment. The bent samples were then allowed to return to room temperature overnight before being subjected to about 0.1 MPa (15 psi) water penetration test per section 3.2.2 of ANSI/ICEA T-31-610-2014. All of the samples passed the test.

Another similar sample cable passed the water penetration test of ICEA S94-649-2013, section 2.2 performed at a water pressure of 0.1 MPa (15 psi) which is greater than the prescribed by said standard, i.e. 0.034 MPa (5 psi).

While the exact water penetration length for each sample was not known, the hot and cold bend tests results confirm that the addition of pulverized crosslinked polymer did not affect the water-blocking compositions ability to impregnated the conductor and efficiently preventing ingress and migration of water in a 1/0 AWG size cable.

Example 2. A cable similar to that of Example 1 (comprising a blend containing a semiconducting thermoplastic water-blocking material and 23.0 wt % of pulverized silane crosslinked polyethylene XLPE with a particle size of about 295 µm) was manufactured and tested except that the blend was applied to a 500 mm<sup>2</sup> (1000 kcm) conductor. Two 0.9 m (36") long sample samples were subjected, respectively, to the hot bend test and the cold bend tests as above, but bent around a 50 cm (20") diameter drum. Both the samples passed the test.

The 500 mm<sup>2</sup> size cable passed the water penetration test of ICEA S94-649-2013, section 2.2 performed at a water pressure of 0.1 MPa (15 psi) which is greater than that prescribed by said standard, i.e. 0.034 MPa (5 psi).

While the exact water penetration length for each sample was not known, the hot and cold bend tests results confirm that the addition of pulverized crosslinked polymer did not affect the water-blocking composition ability to impregnated the conductor and efficiently preventing ingress and migration of water in a 500 mm<sup>2</sup> size cable.

Example 3. A water-blocking composition containing 32.6 wt % of pulverized crosslinked XLPE was used to manufacture a 42.4 mm<sup>2</sup> (1/0 AWG) size cable at various line

## 12

speeds starting from that generally suitable for industrial application, i.e. 450 RPMs. The results are shown below in Table 1.

TABLE 1

| Line Speed (RPMs) | Result                                                               |
|-------------------|----------------------------------------------------------------------|
| 450               | Breakages in the water-blocking material observed.                   |
|                   | Breakages were not alleviated by adjustment of the strand seal pump. |
| 310               | Breakages in the water-blocking material observed                    |
| 278               | Breakages in the water-blocking material observed                    |
| 250               | No breakages observed in the water-blocking material                 |

15 The starting portion of about 300 m (1,000 ft.) manufactured at 450 RPMs was not acceptable due to the excessive amounts of strand seal breaks. The manufacturing speed was progressively slowed down and a portion of about 600 (2,000 ft.) obtained at 250 RPMs was finally acceptable for subsequent testing.

20 As shown in Table 1, concentrations of up to about 33 wt % of the crosslinked XLPE could be incorporated into the virgin water-blocking material so long as the run speed did not exceed 250 RPMs. However, regular cable manufacturing line speeds (i.e., >300 RPMs) could not be used without breakage of the water-blocking material, making a water-blocking composition containing such an amount of pulverized crosslinked polymer unsuitable for an industrially efficient manufacturing process.

25 Example 4 The following additional samples of 1/0 AWG cables were prepared in the same manner as Example 1 except that the mixtures contained 32.6% of pulverized silane crosslinked polyethylene XLPE and that the sample was prepared at a manufacturing speed of 250 RPMs

30 0.9 m (36") long samples of the above were bent around a 20.32 cm (8") diameter drum after performing a 140° C. hot treatment, while other similar samples were bent around a 20.32 cm (8") diameter drum after performing a -10° C. cold treatment. The bent samples were then allowed to return to room temperature overnight before being subjected to about 0.1 MPa (15 psi) water penetration test per section 3.2.2 of ANSI/ICEA T-31-610-2014. While the samples bent under hot treatment passed the water penetration test, one sample out of three samples bent under cold treatment failed the test. A cable with the conductor filled with a water-blocking composition containing an amount of crosslinked polymer greater than 30 wt % should be manufactured at a line speed slower than an industrially acceptable one and showed to be not fully reliable in the presence of water.

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 90

## 13

density polyethylene, crosslinked linear low density polyethylene, crosslinked medium density polyethylene, crosslinked high density polyethylene, ethylene-propylene rubber, ethylene propylene diene rubber, ethylene vinyl acetate, ethylene butyl acetate, ethylene ethyl acetate, or mixtures thereof.

2. The power cable of claim 1, wherein the water-blocking composition comprises at least 10 wt % of the crosslinked polymer based on a total weight of the water-blocking composition.

3. The power cable of claim 1, wherein the water-blocking composition comprises from 10-25 wt % of the crosslinked polymer based on a total weight of the water-blocking composition.

4. The power cable of claim 1, wherein the water-blocking composition comprises from 20-90 wt % of the thermoplastic polymer based on a total weight of the water-blocking composition.

5. The power cable of claim 1, wherein water-blocking composition comprises from 65-85 wt % of the thermoplastic polymer based on a total weight of the water-blocking composition.

6. The power cable of claim 1, wherein the crosslinked polymer is in the form of a powder having a particle diameter from 100  $\mu\text{m}$  to 600  $\mu\text{m}$ .

7. The power cable of claim 6, wherein the crosslinked polymer is in the form of a powder having a particle diameter from 200  $\mu\text{m}$  to 400  $\mu\text{m}$ .

8. The power cable of claim 1, wherein the thermoplastic polymer and/or the crosslinked polymer are semiconductive.

9. The power cable of claim 1, wherein the thermoplastic polymer is selected from the group consisting of a polyeth-

## 14

ylene homopolymer, a polyethylene copolymer, an isobutylene homopolymer, air isobutylene copolymer, a butadiene-styrene copolymer, and an ethyl vinyl acetate polymer.

10. The power cable of claim 1, wherein the crosslinked polymer comprises a fully crosslinked polymer.

11. The power cable of claim 1, wherein the water-blocking material completely fills any interstices of the stranded conductive wire.

12. The power cable of claim 1, wherein the crosslinked polymer is in the form of a powder having a particle diameter from 200 to less than 900  $\mu\text{m}$ .

13. A process for manufacturing a power cable, the process comprising:

15 dispersing a positive amount of up to 30 wt % of a crosslinked polymer in the form of a powder having a particle diameter less than 900  $\mu\text{m}$  in a thermoplastic polymer to obtain a water-blocking composition;

20 pumping the water-blocking composition to impregnate stranded electrically conductive wires, to obtain a cable core.

14. The process of claim 13, wherein the pumping is carried out at a line speed greater than 250 rotations per minute.

25 15. The process of claim 13, wherein, during the pumping, the water-blocking composition is pumped through a heated hose.

30 16. The process of claim 13, wherein the pumping is carried out at a line speed of at least 400 rotations per minute.

\* \* \* \* \*